# EUROPEAN PATENT SPECIFICATION

(11) **EP 4 227 431 B1**
(45) Date of publication and mention of the grant of the patent: **29.07.2026**
(21) Application number: 21847037.5
(22) Date of filing: 14.09.2021
(51) Int. Cl.: C22C 38/00, C22C 38/02, C22C 38/04, C22C 38/12, B22D 11/00, B22D 11/22, C21C 7/06, C21C 7/072

(54) **METHOD FOR PRODUCING V-N MICROALLOYED AND SURFACE-CRACK-FREE CONTINUOUS CASTING BLANK**
VERFAHREN ZUR HERSTELLUNG EINES V-N-MIKROLEGIERTEN UND RISSFREIEN STRANGGUSSROHLINGS
PROCÉDÉ DE PRODUCTION D'UNE ÉBAUCHE DE COULÉE CONTINUE MICROALLIÉE EN V-N ET SANS FISSURE DE SURFACE

(30) Priority: 18.09.2020 CN 202010990234
(43) Date of publication of application: 16.08.2023
(73) Proprietor: Laiwu Steel Yinshan Section Co., Ltd., Ji'nan, Shandong 271104 (CN)
(72) Inventor: WANG, Zhongxue, Ji'nan, Shandong 271104 (CN); HUO, Xiaoxin, Ji'nan, Shandong 271104 (CN); DU, Linxiu, Ji'nan, Shandong 271104 (CN); MA, Heng, Ji'nan, Shandong 271104 (CN); ZHANG, Pei, Ji'nan, Shandong 271104 (CN); SUN, Zhengxu, Ji'nan, Shandong 271104 (CN); DU, Chuanzhi, Ji'nan, Shandong 271104 (CN); GAO, Zhibin, Ji'nan, Shandong 271104 (CN); WU, Hongyan, Ji'nan, Shandong 271104 (CN); HE, Kang, Ji'nan, Shandong 271104 (CN); ZHANG, Qingpu, Ji'nan, Shandong 271104 (CN); YIN, Xunqiang, Ji'nan, Shandong 271104 (CN)
(74) Representative: Murgitroyd & Company
(86) International application number: PCT/CN2021/118337
(87) International publication number: WO 2022/017545

(56) References cited:
- CN-A- 1 405 351
- CN-A- 1 405 351
- CN-A- 109 852 891
- CN-A- 111 996 466
- GB-A- 1 289 373
- US-A- 3 173 782
- YANG YINGDONG ET AL: "Effect of Nitrogen Content Control on Surface Cracks of S450J0-T Hot-rolled H-shaped steel", SHANGHAI JINSHU, vol. 40, no. 3, 31 May 2018 (2018-05-31), CN, pages 69 - 72, XP055889397, ISSN: 1001-7208
- YANG YINGDONG, CHUNLIN HU, JIAN WU, YINBO TANG, LEI SHI, JIE LI: "Effect of Nitrogen Content Control on Surface Cracks of S450J0-T Hot-rolled H-shaped steel ", SHANGHAI JINSHU, SHANGHAISHI YOUSE JINSHU XUEHUI, CN, vol. 40, no. 3, 31 May 2018 (2018-05-31), CN , pages 69 - 72, XP055889397, ISSN: 1001-7208

## Description

### FIELD OF THE INVENTION

The present invention belongs to the field of continuous casting technology and specifically relates to a method for producing V-N microalloyed and surface-crack-free continuous casting blank.

### BACKGROUND OF THE INVENTION

Microalloyed steel is a kind of rapidly developing steel for engineering structures in nearly past half century. It plays a role in fine-grain strengthening and precipitation strengthening by adding various alloy elements (Nb, V, Ti, etc.) to the steel, thus improvingthe strength and toughnessof the steel. It is widely used in various fields for example bridges, buildings, ships, automobiles, high-pressure vessels, etc., and has good application prospects. It is the main product in the modern steel industry. China has abundant reserves of microalloyed elements and has significant advantages in developing microalloyed steel. Typical Q550 and Q460grades low content alloy high-strength steel have good market applications.

GB1289373A discloses a process for manufacturing a killed, low-alloy, high-strength steel consisting of at least 0.12% carbon, a maximum of 1.65% manganese, at least 0.05% vanadium, 0.005% to 0.025% nitrogen, 0.04% maximum phosphorus, 0.025% maximum sulphur, 0.60% maximum silicon, aluminium in an amount sufficient to provide a killed steel, balance iron (and unavoidable impurities). Its process comprises hot-rolling the steel and finishing at a temperature of 1550°F to 1650°F, thereafter cooling the hot-rolled steel at a rate of 20°F to 135°F per second to a temperature of 1025°F to 1175°F.

In the industrial production process, microalloying is widely used due to the strengthening effect of microalloying elements. However, during the continuous casting process, the carbonitride precipitation of microalloying elements reduces the plasticity of steel, and the occurrence rate of surface cracks in continuous casting billets is significantly higher than that of ordinary carbon steel casting blank. There are problems for example transverse cracks, longitudinal cracks, and shape cracks, so as to affect the quality of continuous casting billets and are not conducive to large-scale productions, which is a typical problem with microalloyed casting blank. Niobium, vanadium, and titanium are three relatively widely used elements in microalloyed steel, with niobium having the greatest impact on the plasticity of the steel and the most significant reduction in its thermoplastic properties.Researches have shown that the addition of Ti elementcan reduce the brittleness of niobium and vanadium microalloyed steels, but it is not easy to control costs.

Therefore, taking into account both cost and the issue of cracks in microalloyed steel casting blanks, developing a low-cost, crack free production process for casting blanks is a typical process difficulty, which not only ensures the performance of microalloyed steel, ensures the normal operation of the continuous casting process, but also improves the surface quality of the casting blanks.

### SUMMARY

In response to the problem of prone to cracks on the surfaces of microalloyed steel casting blanks during continuous casting in existing technologies, the present invention provides a method for producing a V-N microalloyed steel of surface-crack-free continuous casting blanks . Through reasonable composition design and smelting **and continuous** casting process, a surface crack free continuous casting blanks with a cross-section of (150-350) mm * (1250-2400) mm is produced, which improves the surface quality of the continuous casting blanks.

To achieve the above objectives, the technical solution adopted by the present invention is as follows:
The present invention takesthe features of the lowvalley point of thermoplastic properties of vanadium containing steel, the chemical composition of microalloyed steel is reasonably designed, so as to reduce the occurrence of surface cracks on the casting blanks during continuous casting.

In the present invention, the V element has a very strong affinity with the N element, and combined with TMCP method in the later stage can play the role of increasing the strength and toughness of the structure through two typical strengthening mechanisms, fine grain strengthening and precipitation strengthening.

At the same time, some regions in China have abundant reserves of vanadium deposit, for example Chengde and Panzhihua, which have good cost advantages, and the price of N is relatively low. Therefore, using V-N microalloying is beneficial for reducing the production cost of continuous casting blanks.

The present invention provides a production method for V-N microalloyed surface-crack-free continuous casting blanks, wherein the casting blanks are produced according to the V-N microalloyed steel consisting of the following chemical componentsby mass percentage: C: 0.09~0.13%, Si: 0.1~0.4%, Mn: 1.0~3.0%, P: ≤ 0.05%, S: ≤ 0.05%, V: 0.1~0.4%, N: 0.011~0.2%, and the balance of Fe and unavoidable impurity elements; and the method sequentially includes the following processes: converter smelting, LF refining, and continuous casting; in the converter smelting process, amolten **ironproportion** is controlled between 88.0 wt% ~ 91.0 wt%, a top-bottom combined blowing mode is used throughout entire process, and nitrogen gas is blown first and then argon gas is blown later during blowing process, wherein an argon-blowing time is not less than 3 minutes; deoxidation alloying is carried out during tapping process in the converter smelting process, while slag filtratingis also carried out;a specific operation method of the deoxidation alloying is as follows:during tapping process, a silicon containing substance is selected for deoxidation with an addition amount of 3.5~4.0kg/ton of steel; and silicon manganese and vanadium nitrogen alloys are selected for alloying, wherein an addition amount ofthe vanadium nitrogen alloyis 1~2 kg/ton of steel;LF refining is performed after tapping,and the refining is without vacuum degassing;in the LF refining process, in an early stage of LF refining, an argon-blowing amount forargon-blowing stirringis 400~1000 L/minute, an argon-blowing stirring time is 3~4 minutes, a silicon containing substance should be used for deoxidation, and the components arefine-tunedunder the condition of argon-blowing stirring;in the LF refining process, at the end of LF refining, an argon-blowing amount for argon-blowing stirring is 100~200 L/minute, and a time of argon-blowing stirring is ≥ 5 minutes; a total refining time is controlled within 40~50 minutes, and N contentobtained is 100~2000ppm;in the continuous casting process,an specific amount of water in the continuous casting process is 0.7~1.25L/kg; in the continuous casting process, protective casting is adopted, water port is closed immediately while large ladle alarms at the end of casting,reopening the water port is strictly prohibited after the water portis closed,an intermediate ladle is covered with alkaline covering agent, anda crystallizer uses low-carbon steel protective slag.

In the above production method, as a preferred embodiment **(mode),** the cross-sectional specification of the continuous casting blank is (150-350) mm * (1250-2400) mm.

In the above production method, in the converter smelting process, the molten iron proportion is controlled between 88.0% ~ 91.0% (for example, 88.0%, 89.0%, 90.0%, and 91.0%), and the top-bottom combined blowing mode is used throughout the entire process, and nitrogen gas is blown first and then argon gas is blown later during the blowing process, to stir the molten steel and promote the chemical reaction in the furnace. Wherein, the argon blowing time is not less than 3 minutes (for example, 3 minutes, 5 minutes, 10 minutes, and 15 minutes).

In the above production method, as a preferred embodiment, in the converter smelting process, the blowing process adopts a one blow to end (one shot to bottom) blowing method without reblowing (supplementary blowing) process, so as to avoid excessive oxidation of molten steel and increase of inclusions during the reblowing process.

In the above production method, as a preferred embodiment, in the converter smelting process, the C content at the smelting endpoint is controlled between 0.09% ~ 0.13% (for example, 0.09%, 0.10%, 0.11%, 0.12%, and 0.13%), and the tapping temperature is between 1625 ~ 1645 °C (for example, 1625 °C, 1630 °C, 1635 °C, 1640 °C, and 1645 °C). The tapping temperature is determined based on the solidification temperature of the molten steel, the degree of superheat during the continuous casting process, and the process temperature drop, so as to ensure the smooth pouring of the continuous casting.

In the above production method, LF refining is performed after tappingwithout vacuum degassing; the purpose of not performing vacuum degassing is to ensure the content of N in the molten steel.

In the above production method, the specific water flow of the **continuous** casting process is 0.7~1.25L/kg (for example, 0.7L/kg, 0.8L/kg, 1.0L/kg, 1.2L/kg, and 1.25L/kg), so as to effectively reduce the occurrence of cracks on the casting blanks.

In the above production method, in the continuous casting process, protective casting is adopted, and the large ladle alarms at the end of casting and thus immediately close the nozzle. After the water portis closed, it is strictly prohibited to open it again. The intermediate ladle is covered with alkaline covering agent to ensure good liquid level coverage, and the crystallizer uses low-carbon steel casting powder.

In the above production method, as a preferred embodiment, in the continuous casting process, the degree of superheat of the continuous casting furnace is strictly controlled, and the degree of superheat of the molten steel is 10~25 °C (for example, 10 °C, 15 °C, 20 °C, and 25 °C).

In the above production method, as a preferred embodiment, in the continuous casting process, the casting speed is 1.0~1.3 m/minutes (for example, 1.0m/minute, 1.1m/minute, 1.2m/minute, and 1.3m/minute).

The control of low degree of superheat in the present invention is beneficial for improving casting speed (drawing speed), shortening pouring time, and reducing energy consumption; the tundish adopts alkaline covering agent to insulate the steel ladle and remove impurities from the steel ladle.

In the above production method, as a preferred embodiment, the protective slag in the continuous casting process is divided into powder slag layer, sintered layer, and liquid slag layer during the dissolution process.

In the above production method, deoxidation alloying is carried out during the tapping process in the converter smelting process, while slag washingis also carried out.

In the above production method, the specific operation method of deoxidation alloying during the tapping process in the converter smelting process is:during the tapping process, silicon containing substances are selected for deoxidation, with an addition amount of 3.5~4.0kg/ton of steel (for example, 3.5kg/ton of steel, 3.6kg/ton of steel, 3.8kg/ton of steel, and 4.0kg/ton of steel); silicon manganese and vanadium nitrogen alloys are selected for alloying, wherein the vanadium nitrogen alloy (V content not less than 75%) is added in amount of 1~2 kg/ton of steel (for example, 1kg/ton of steel, 1.2kg/ton of steel, 1.4kg/ton of steel, 1.6kg/ton of steel, 1.8kg/ton of steel, 2kg/ton of steel). The present invention does not use aluminum for deoxidation.

In the above production method, as a preferred embodiment, during the tapping process in the converter smelting process, the slag filtrating (washing) is carried out using a substance containing CaO (with a CaO content of not less than 90%), with an addition amount of 3.5~4.0kg/ton of steel (for example, 3.5kg/ton of steel, 3.6kg/ton of steel, 3.8kg/ton of steel, and 4.0kg/ton of steel). The substance containing CaO needs to be added before the molten steel reaches 3/4.

In the above production method, during the LF refining, in the early stage of LF refining, the argon blowing amount of argon stirringis 400~1000 L/minute (for example, 500 L/minute, 600 L/minute, 700 L/minute, 800 L/minute, and 900 L/minute), and the argon stirring time is 3~4 minutes (for example, 3 minutes, 3.2 minutes, 3.5 minutes, 3.8 minutes, and 4 minutes). During stirring, attention should be paid to not exposing the molten steel.And then silicon containing substances should be used for deoxidation,andfine tune the composition under the condition of argon stirring.

In the above production method, as a preferred embodiment, **during** the LF refining, weak argon stirring is adopted in the middle stage and end stage of LF refining, with the same argon blowing flow rate.

In the above production method, during the LF refining, in the end stage of LF refining,the argon blowing amount of argon stirring is 100~200 L/minute (for example, 120 L/minute, 140 L/minute, 160 L/minute, and 180 L/minute), and the time of argon stirring is ≥ 5 minutes; the total refining time is controlled within 40~50 minutes (for example, 40 minutes, 42 minutes, 45 minutes, 48 minutes, and 50 minutes), and the obtained N content is 100~2000ppm (for example, 100ppm, 500ppm, 1000ppm, 1500ppm, 2000ppm). The other component content meets the required molten steel composition content in the smelting process.

In the continuous casting process of the present invention, the different water volumedistribution is selected based on the different specifications of the casting blanks and the composition of the steel grade duringthe continuous casting process.

In the above production method, as a preferred embodiment, during the continuous casting process, the specific distribution of water volume in the continuous casting process is as follows: the water volume in the inner and outer arcs of the wide-side foot-roller of the casting blank accounts for 8.0~10.0% of the total water volume (for example, 8.0%, 8.5%, 9.0%, 9.5%, and 10.0%), the water volume in the narrow-side foot-roller accounts for 3.4~4.5% of the total water volume (for example, 3.4%, 3.8%, 4.0%, 4.2%, and 4.5%), and the water volume in the inner and outer arcs of the second zone of the vertical bending section accounts for 11.0~15.9% of the total water volume (for example, 11.0%, 12.0%, 13.0%, 14.0%, 15.0%, 15.5%, and 15.9%), the water volume in the inner and outer arcs of the third zone accounts for 13.0~15.9% of the total water volume (for example, 13.0%, 14.0%, 15.0%, 15.5%, and 15.9%), the water volume in the inner and outer arcs of the fourth zone accounts for 12.0~13.0% of the total water volume (for example, 12.0%, 12.2%, 12.5%, 12.6%, 12.8%, and 13.0%), the water volume in the inner and outer arcs of the fifth zone of arc section 1 accounts for 8.5~9.5% of the total water volume (for example, 8.0%, 8.5%, 9.0%, and 9.5%), the water volume in the inner and outer arcs of the sixth zone corresponding to arc sections 2 and 3 accounts for 12.0~14.0% of the total water volume (for example, 12.0%, 12.5%, 13.0%, 13.5%, 13.8%, and 13.0%), the water volume in the inner and outer arcs of the seventh zone of the sections 4~5 accounts for 8.0~11.5% of the total water volume (for example, 8.0%, 8.5%, 9.0%, 9.5%, 10.0%, 11.0%, 11.5%, and 10.0%),the water volume in the inner and outer arcs of the eighth zone of the straightening sections 6, section 7 and section 8 accounts for 8.0~11.5% of the total water volume (for example, 8.0%, 8.5%, 9.0%, 9.5%, 10.0%, 11.0%, 11.5%, and 10.0%),while the remaining water volume is allocated to the horizontal section.

In the present invention, the above technical features can be freely combined to form new technical solutions without conflicting with each other.

The steps and processes not detailed in the production methods provided by the present invention are conventional processes in the art.

Compared with the prior art, the beneficial effects of the present invention are:
the production method for V-N microalloyed and surface-crack-free continuous casting blank presented by the invention improves the thermoplastic properties of the continuous casting blanks through reasonable composition design of V-N microalloying, combined with appropriate smelting and continuous casting processes,avoiding high-temperature brittle zones or having sufficient thermoplastic properties in the straightening range of the blanks to prevent surface cracks from occurring. The surface quality of the billets is good, without the need for cleaning the casting blanks, and the production efficiency is improved.

### DETAILED DESCRIPTION OF THE EMBODYMENTS

The following will provide a detailed explanation of the technical solution of the present invention in conjunction with embodiments. Each example is provided through the interpretation of the present invention rather than limiting it. In fact, those skilled in the art will be aware that modifications and variations can be made in the present invention without departing from the scope of the present invention. For example, features shown or described as part of one embodiment may be used in another embodiment to generate another embodiment. Therefore, it is expected that the present invention includes such modifications and variations within the scope of the accompanying claims.

According to the embodiment of the present invention, it provides a method for producing a surface-crack-free continuous casting blanks V-N microalloyed steel. The V-N microalloyed steel is composed of the following chemical componentsby mass percentage: C: 0.09~0.13%, Si: 0.1~0.4%, Mn: 1.0~3.0%, P: ≤ 0.05%, S: ≤ 0.05%, V: 0.1~0.4%, N: 0.011~0.2%, and the balance of Fe and a small amount of unavoidable impurity elements. The present invention provides a production method for preparing surface-crack-free microalloyed steel for continuous casting blanks with the above-mentioned chemical components,the method sequentially includes the following processes: converter smelting, LF refining, and continuous casting; in the converter smelting process, amolten ironproportion is controlled between 88.0 wt% ~ 91.0 wt%, a top-bottom combined blowing mode is used throughout entire process, and nitrogen gas is blown first and then argon gas is blown later during blowing process, wherein an argon-blowing time is not less than 3 minutes; deoxidation alloying is carried out during tapping **process** in the converter smelting process, while slag filtratingis also carried out;a specific operation method of the deoxidation alloying is as follows:during tapping process, a silicon containing substance is selected for deoxidation with an addition amount of 3.5~4.0kg/ton of steel; and silicon manganese and vanadium nitrogen alloys are selected for alloying, wherein an addition amount ofthe vanadium nitrogen alloyis 1~2 kg/ton of steel;LF refining is performed after tapping,and the refining is without vacuum degassing;in the LF refining process, in an early stage of LF refining, an argon-blowing amount forargon-blowing stirringis 400~1000 L/minute, an argon-blowing stirring time is 3~4 minutes, a silicon containing substance should be used for deoxidation, and the components arefine-tunedunder the condition of argon-blowing stirring;in the LF refining process, at the end of LF refining, an argon-blowing amount for argon-blowing stirring is 100~200 L/minute, and a time of argon-blowing stirring is ≥ 5 minutes; a total refining time is controlled within 40~50 minutes, and N contentobtained is 100~2000ppm;in the continuous casting process,an specific amount of water in the continuous casting process is 0.7~1.25L/kg; in the continuous casting process, protective casting is adopted, water port is closed immediately while large ladle alarms at the end of casting,reopening the water port is strictly prohibited after the water portis closed,an intermediate ladle is covered with alkaline covering agent, anda crystallizer uses low-carbon steel protective slag.

The alkaline covering agent and low-carbon steel protective slag used in the production process of the continuous casting blank of the present invention are commonly used commercial products for producing microalloyed steel.

Due to the carbonitride precipitates during continuous casting process, the plasticity of steel is decreased, the occurrence rate of surface cracks of continuous casting blank is significantly higher than that of ordinary carbon steel blank, and problems such as transverse cracks, longitudinal cracks, and shape cracks occur. In the smelting process of the invention,the contents of C are controlled, S is reduced, the use of a deoxidant is controlled, the inclusion morphology is changed, and the purity of steel is improved.In combination with LF refining and reasonable continuous casting process, a microalloyed steel with fine grains and good plasticity is obtained, thereby reducing the occurrence of surface cracks in a continuous casting blank of microalloyed steel , improving the surface quality of a continuous casting blank.

### Example 1

This example provides a V-N microalloyed continuous casting blank and its production method, and the chemical composition of the continuous casting blank is shown in Table 1 by mass percentage.

**Table 1 The chemical component of the V-N microalloyed continuous casting blank from Example 1**

| Example | chemical component(wt%), the balance of Fe and unavoidable impurity elements | | | | | | |
|---|---|---|---|---|---|---|---|
| | C | Si | Mn | P | S | V | N |
| 1 | 0.10 | 0.23 | 1.62 | 0.014 | 0.007 | 0.12 | 0.012 |

The production method sequentially includes the following processes: converter smelting, LF refining and continuous casting.
(1) Converter smelting:
   During a converter smelting process, a 120t converter is used for smelting,the smelting raw materials are molten iron and steel scrap, and the ratio of molten iron is controlled at 90%;nitrogen gas is used for blowing in the early stage of blowing and argon gas used for blowing in the later stage with4 minutes of the argon gas blowing, and a gun-to-bottom type for blowingis carried out in the blowing process, absolutely eliminating the supplementary blowing process, thereby preventing the molten steel from being peroxided so as to improvethe cleanliness of the molten steel.
   The C content at the smelting endpoint is controlled at 0.10wt%, and the tapping temperature is 1632 °C; deoxidation alloying and slag filtrating are carried out during tapping, silicon containing material is selected as deoxidizing agent with the addition amount of about 3.6kg/t steel; the alloyed raw material is vanadium nitrogen alloy (with a V content of 77wt%) with an addition of about 1.6kg/ton of steel; and a substance containing CaO is selected for slag filtrating(with a CaO content of 90wt%) with an added amount of 3.8kg/ton of steel.
(2)LF refining:
   The steel ladle is directly transferred to the LF refining station for argon blowing refining after tapping;in the early stage of refining, the argon blowing rate at400L/minute is selected for argon blowingstirring for 3 minutes ,then silicon containing substances are added for deoxygenation, and a small amount of silicon manganese is added to adjust the Mn content; at the end stage of refining, the argon blowing rate is adjusted to 150L/minute and stirred for 6 minutes; the total refining time is controlled at 45 minutes, the N content obtained is 120 ppm andthe content of other components meets the requirements of molten steel composition in the composition control process.
(3)Continuous casting:
   In the protective casting process, the large ladle is protected with a long water port and a conical asbestos pad is added to ensure the air-tightness of the connection.

After the casting starts, a coal gas flame is firstly used to check air-tightness of the lower water port of the ladleand the bowl part of long water port. If the flame is sucked in, it indicates poor sealing at this location, and a new long water portis jointed. If the air-tightness meets the requirements, argon gas is introduced into the bowl part **connection** of the long water portto form an argon sealing stateduring the pouring process, further preventing oxygen and nitrogen increase in the molten steelcaused by the loose connection between the bowl part of long water portand the lower water portof the ladle due to air intake .

Immediately close the water port when the large ladle alarmed at the end of pouring. It is strictly prohibited to reopen the water portafter it is closed. The tundish is covered with alkaline covering agent, and the crystallizer is protected with low-carbon steel protective slag (special P0050 of Shinagawa 250).

This example is the third furnace for casting, that is,a third furnace steel which is cast after the start of continuous casting. The degree of superheat is 20 °C, and the actual drawing speed is 1.1m/minute.

During the continuous casting process, the specific distribution of water volume with a specific water flow (specific amount of water) of 1.2L/kgis as follows: the amount of water in the inner and outer arcs of the wide-side foot-roller of the casting blank accounts for about 8.6% of the total amount ofwater, the amount of water in the narrow-side foot-roller accounts for 3.5% of the total amount of water, and the amount of water in the inner and outer arcs of the second zone of the vertical bending section accounts for 15.8% of the total amount of water, the water volume in the inner and outer arcs of the third zone accounts for 15.6% of the total water volume, the water volume in the inner and outer arcs of the fourth zone accounts for 12.9% of the total water volume, the water volume in the inner and outer arcs of the fifth zone of arc section 1 accounts for 9.3% of the total water volume, the water volume in the inner and outer arcs of the sixth zone corresponding to arc sections 2 and 3 accounts for 12.4% of the total water volume, the water volume in the inner and outer arcs of the seventh zoneof the sections 4~5 accounts for 8.1% of the total water volume,the water volume in the inner and outer arcs of the eighth zone of the straightening sections 6, section 7 and section 8 accounts for 8.9% of the total water volume,while the remaining water volume is allocated to the horizontal section.

Implementation effect: The continuous casting blank obtained from the multi furnace steel cast by the above method has a cross-sectional area of 200mm * 2000mm, good surface quality, no cracks detected at low magnification, and no cracks observed on the surface of the casting blank during hot state observation, without the need for casting blank cleaning.

### Example 2

This example provides a V-N microalloyed continuous casting blank, and the chemical composition of the continuous casting blank is shown in Table 2 by mass percentage.

**Table 2 The chemical component of the V-N microalloyed continuous casting blank from Example 2**

| Example | chemical component(wt%), the balance of Fe and unavoidable impurity elements | | | | | | |
|---|---|---|---|---|---|---|---|
| | C | Si | Mn | P | S | V | N |
| 2 | 0.09 | 0.40 | 1.00 | 0.014 | 0.006 | 0.25 | 0.032 |

The production method sequentially includes the following processes: converter smelting, LF refining, and continuous casting.

### (1) Converter smelting:

During a converter smelting process, a 120t converter is used for smelting,the smelting raw materials are molten iron and steel scrap, and the ratio of molten iron is controlled at 89%;nitrogen gas is used for blowing in the early stage of blowing and argon gas used for blowing in the later stage with3 minutes of the argon gas blowing, and **a gun-to-bottom** type for blowing is carried out in the blowing process, absolutely eliminating the supplementary blowing process .

The C content at the smelting endpoint is controlled at 0.09t%, and the tapping temperature is 1630 °C.

Deoxidation alloying and slag filtrating are carried out during tapping, and silicon containing material is selected as deoxidizing agent(that is,silicon carbide) with the addition amount of about 3.8kg/t steel; the alloyed raw material is vanadium nitrogen alloy (with a V content of 77wt%) with an addition of about 1.3kg/ton of steel; and a substance containing CaO is selected for slag filtrating(with a CaO content of 90wt%) with an added amount of 3.6kg/ton of steel.

### (2)LF refining:

The steel ladle is directly transferred to the LF refining station for argon blowing refining after tapping,in the early stage of refining,the argon blowing rate at 400L/minute is selected for argon blowing stirring for 4 minutes,andthen silicon containing substances are added for deoxygenation; at the end stage of refining, the argon blowing rate is adjusted to 150L/minute and stirred for 7 minutes; the total refining time is controlled at 48 minutes, the N content obtained is 100 ppm, and the content of other components meets the requirements of molten steel composition in the composition control process.

### (3)Continuous casting:

In the protective casting process, the large ladle is protected with a long water portand a conical asbestos pad is added to ensure the air-tightness of the connection.After the casting starts, a coal gas flame is firstly used to check air-tightness of the lower water portand the bowl part of the long water port. If the flame is sucked in, it indicates poor sealing at this location, and a new long water portis jointed. If the air-tightness meets the requirements, argon gas is introduced into the bowl part connection of the long water portto form an argon sealing stateduring the pouring process, further preventing oxygen and nitrogen increase in the molten steel caused by the loose connection between the long water portbowl part and the lower water portof the ladle due to air intake.Immediately close the water port when the large ladle alarmedat the end of pouring. It is strictly prohibited to reopen the water portafter it is closed. The tundish is covered with alkaline covering agent, and the crystallizer is protected with low-carbon steel protective slag (special P0027-3of Shinagawa 250).

This example is the fourth furnace of steel poured after the continuous casting start. The degree of superheat is 15 °C, and the actual drawing speed is 1.2m/minute.

During the continuous casting process, the specific distribution of water volume with a specific water flow of 1.0L/kg is as follows: the water volume in the inner and outer arcs of the wide-side foot-roller of the casting blank accounts for about 8.1% of the total water volume, the water volume in the narrow-side foot-roller accounts for 4.3% of the total water volume, and the water volume in the inner and outer arcs of the second zone of the vertical bending section accounts for 11.4% of the total water volume, the water volume in the inner and outer arcs of the third zone accounts for 13.1% of the total water volume, the water volume in the inner and outer arcs of the fourth zone accounts for 12% of the total water volume, the water volume in the inner and outer arcs of the fifth zone of arc section 1 accounts for 9.0% of the total water volume, the water volume in the inner and outer arcs of the sixth zone corresponding to arc sections 2 and 3 accounts for 13.6% of the total water volume, the water volume in the inner and outer arcs of the seventh zone of the sections 4~5 accounts for 11.2% of the total water volume,the water volume in the inner and outer arcs of the eighth zoneof the straightening sections 6, section 7 and section 8 accounts for 11.3% of the total water volume,while the remaining water volume is allocated to the horizontal section.

Implementation effect: The continuous casting blank obtained from the multi furnace steel cast by the above method has a cross-sectional area of 250mm * 1800mm, good surface quality, no cracks detected at low magnification, and no cracks observed on the surface of the casting blank during hot state observation, without the need for casting blank cleaning.

The above is only a preferred embodiment of the present invention and is not intended to limit the present invention. For those skilled in the art, the present invention may undergo various modifications and variations within the scope of the invention as defined in the appended claims.

## Claims

1. A production method for V-N microalloyed surface-crack-free continuous casting blanks, **characterized in that** the casting blanks are produced according to the V-N microalloyed steel consisting of the following chemical componentsby mass percentage: C: 0.09~0.13%, Si: 0.1~0.4%, Mn: 1.0~3.0%, P: ≤ 0.05%, S: ≤ 0.05%, V: 0.1~0.4%, N: 0.011~0.2%, and the balance of Fe and unavoidable impurity elements; the method includes the following processes in sequence: converter smelting, LF refining and continuous casting;
in the converter smelting process, a molten iron proportion is controlled between 88.0 wt% ~ 91.0 wt%, a top-bottom combined blowing mode is used throughout entire process, and nitrogen gas is blown first and then argon gas is blown later during blowing process, wherein an argon-blowing time is not less than 3 minutes;
deoxidation alloying is carried out during tapping process in the converter smelting process, while slag filtratingis also carried out; a specific operation method of the deoxidation alloying is as follows: during tapping process, a silicon containing substance is selected for deoxidation with an addition amount of 3.5~4.0kg/ton of steel; and silicon manganese and vanadium nitrogen alloys are selected for alloying, wherein an addition amount ofthe vanadium nitrogen alloyis 1~2 kg/ton of steel;
LF refining is performed after tapping, and the refining is without vacuum degassing;
in the LF refining process, in an early stage of LF refining, an argon-blowing amount for argon-blowing stirring is 400~1000 L/minute, an argon-blowing stirring time is 3~4 minutes, a silicon containing substance should be used for deoxidation, and the components are fine-tuned under the condition of argon-blowing stirring;
in the LF refining process, at the end of LF refining, an argon-blowing amount for argon-blowing stirring is 100~200 L/minute, and a time of argon-blowing stirring is ≥ 5 minutes; a total refining time is controlled within 40~50 minutes, and N contentobtained is 100~2000ppm;
in the continuous casting process, an specific amount of water in the continuous casting process is 0.7~1.25L/kg; in the continuous casting process, protective casting is adopted, water port is closed immediately while large ladle alarms at the end of casting, reopening the water port is strictly prohibited after the water portis closed, an intermediate ladle is covered with alkaline covering agent, and a crystallizer uses low-carbon steel protective slag.

2. The production method according to claim 1, **characterized in that** a cross-sectional specification of the continuous casting blanks is (150-350) mm * (1250-2400) mm.

3. The production method according to claim 1 or claim 2, **characterized in that** in the converter smelting process, the blowing process adopts a one blow to end blowing mode without reblowing process;
preferably, a C content at smelting endpoint is controlled between 0.09 ~ 0.13wt%, and a tapping temperature is between 1625 ~ 1645 °C.

4. The production method according to claim 1, **characterized in that** in the continuous casting process,a superheatdegree of molten steel is 10~25 °C ;
preferably, a casting speed during continuous casting process is 1.0~1.3 m/minute.

5. The production method according to claim 1, **characterized in that** the slag filtrating is carried out using a substance containing CaO with an addition amount of 3.5~4.0kg/ton of steel, and the substance containing CaO needs to be added before molten steel reaches 3/4.

6. The production method according to claim1, **characterized in that** in the continuous casting process, a specific distribution of water volume in the continuous casting process is as follows: a water volume in inner and outer arcs of a wide-side foot-roller of the casting blank accounts for 8.0~10.0% of the total water volume, awater volume in a narrow-side foot-roller accounts for 3.4~4.5% of the total water volume, and a water volume in inner and outer arcs of a second zone of a vertical bending section accounts for 11.0~15.9% of the total water volume, a water volume in inner and outer arcs of a third zone accounts for 13.0~15.9% of the total water volume, a water volume in inner and outer arcs of a fourth zone accounts for 12.0~13.0% of the total water volume, a water volume in inner and outer arcs of a fifth zone of arc section 1 accounts for 8.5~9.5% of the total water volume, a water volume in inner and outer arcs of a sixth zone corresponding to arc sections 2 and 3 accounts for 12.0~14.0% of the total water volume, a water volume in inner and outer arcs of a seventh zone of sections 4~5 accounts for 8.0~11.5% of the total water volume, a water volume in inner and outer arcs of a eighth zone of straightening section 6, section 7 and section 8 accounts for 8.0~11.5% of the total water volume, and a remaining water volume is allocated to a horizontal section.

## Patentansprüche

1. Herstellungsverfahren für V-N-mikrolegierte, oberflächenrissfreie Stranggussrohlinge, **dadurch gekennzeichnet, dass** die Gussrohlinge aus einem V-N-mikrolegierten Stahl hergestellt werden, der aus den folgenden chemischen Bestandteilen in Massenprozent besteht: C: 0,09-0,13 %, Si: 0,1-0,4 %, Mn: 1,0-3,0 %, P: ≤ 0,05 %, S: ≤ 0,05 %, V: 0,1-0,4 %, N: 0,011~0,2 % und dem Rest Fe und unvermeidbaren Verunreinigungselementen; wobei das Verfahren nacheinander die folgenden Prozesse umfasst: Konverter-Schmelzen, LF-Raffinieren und Stranggießen; wobei im Konverter-Schmelzprozess ein Roheisenanteil zwischen 88,0 Gew.-% und 91,0 Gew.-% gesteuert wird, über den gesamten Prozess hinweg ein kombiniertes Auf- und Bodenblasverfahren angewendet wird und während des Blasprozesses zuerst Stickstoffgas und später Argongas geblasen wird, wobei eine Argonblaszeit nicht weniger als 3 Minuten beträgt; wobei eine Desoxidationslegierung während des Abstichprozesses im Konverter-Schmelzprozess durchgeführt wird, während auch eine Schlackefiltration durchgeführt wird; wobei ein spezifisches Betriebsverfahren der Desoxidationslegierung wie folgt ist: während des Abstichprozesses wird eine siliciumhaltige Substanz zur Desoxidation mit einer Zugabemenge von 3,5~4,0 kg/Tonne Stahl ausgewählt; und Silicium-Mangan- und Vanadium-Stickstoff-Legierungen werden zum Legieren ausgewählt, wobei eine Zugabemenge der Vanadium-Stickstoff-Legierung 1~2 kg/Tonne Stahl beträgt; wobei das LF-Raffinieren nach dem Abstich durchgeführt wird und das Raffinieren ohne Vakuumentgasung erfolgt; wobei im LF-Raffinierungsprozess in einer frühen Phase des LF-Raffinierens eine Argonblasmenge zum Rühren durch Argonblasen 400-1000 L/Minute beträgt, eine Rührzeit durch Argonblasen 3~4 Minuten beträgt, eine siliciumhaltige Substanz zur Desoxidation verwendet werden sollte und die Komponenten unter der Bedingung des Rührens durch Argonblasen feingestellt werden; wobei im LF-Raffinierungsprozess am Ende des LF-Raffinierens eine Argonblasmenge zum Rühren durch Argonblasen 100-200 L/Minute beträgt und eine Zeit des Rührens durch Argonblasen ≥ 5 Minuten beträgt; eine Gesamtraffinierungszeit innerhalb von 40-50 Minuten gesteuert wird und der erhaltene N-Gehalt 100-2000 ppm beträgt; wobei im Stranggussprozess eine spezifische Wassermenge im Stranggussprozess 0,7~1,25 L/kg beträgt; wobei im Stranggussprozess ein Schutzguss angewendet wird, ein Ausguss sofort geschlossen wird, wenn die Gießpfanne am Ende des Gießens Alarm schlägt, ein erneutes Öffnen des Ausgusses strengstens verboten ist, nachdem der Ausguss geschlossen wurde, ein Zwischenverteiler mit einem alkalischen Abdeckmittel abgedeckt wird und eine Kokille kohlenstoffarme Stahlschutzschlacke verwendet.

2. Herstellungsverfahren nach Anspruch 1, **dadurch gekennzeichnet, dass** eine Querschnittsspezifikation der Stranggussrohlinge (150-350) mm * (1250-2400) mm beträgt.

3. Herstellungsverfahren nach Anspruch 1 oder 2, **dadurch gekennzeichnet, dass** im Konverter-Schmelzprozess der Blasprozess ein Einmaldurchblasverfahren bis zum Ende ohne Nachblasprozess anwendet; vorzugsweise ein C-Gehalt am Schmelzendpunkt zwischen 0,09 und 0,13 Gew.-% gesteuert wird und eine Abstichtemperatur zwischen 1625 und 1645 °C liegt.

4. Herstellungsverfahren nach Anspruch 1, **dadurch gekennzeichnet, dass** im Stranggussprozess ein Überhitzungsgrad des geschmolzenen Stahls 10-25 °C beträgt; vorzugsweise eine Gießgeschwindigkeit während des Stranggussprozesses 1,0~1,3 m/Minute beträgt.

5. Herstellungsverfahren nach Anspruch 1, **dadurch gekennzeichnet, dass** die Schlackefiltration unter Verwendung einer CaO-haltigen Substanz mit einer Zugabemenge von 3,5~4,0 kg/Tonne Stahl durchgeführt wird und die CaO-haltige Substanz zugegeben werden muss, bevor der geschmolzene Stahl 3/4 erreicht.

6. Herstellungsverfahren nach Anspruch 1, **dadurch gekennzeichnet, dass** im Stranggussprozess eine spezifische Verteilung des Wasservolumens im Stranggussprozess wie folgt ist: ein Wasservolumen in inneren und äußeren Bögen einer breitseitigen Fußrolle des Gussrohlings macht 8,0∼10,0 % des Gesamtwasservolumens aus, ein Wasservolumen in einer schmalseitigen Fußrolle macht 3,4~4,5 % des Gesamtwasservolumens aus, ein Wasservolumen in inneren und äußeren Bögen einer zweiten Zone eines vertikalen Biegeabschnitts macht 11,0~15,9 % des Gesamtwasservolumens aus, ein Wasservolumen in inneren und äußeren Bögen einer dritten Zone macht 13,0~15,9 % des Gesamtwasservolumens aus, ein Wasservolumen in inneren und äußeren Bögen einer vierten Zone macht 12,0~13,0 % des Gesamtwasservolumens aus, ein Wasservolumen in inneren und äußeren Bögen einer fünften Zone des Bogenabschnitts 1 macht 8,5~9,5 % des Gesamtwasservolumens aus, ein Wasservolumen in inneren und äußeren Bögen einer sechsten Zone entsprechend den Bogenabschnitten 2 und 3 macht 12,0~14,0 % des Gesamtwasservolumens aus, ein Wasservolumen in inneren und äußeren Bögen einer siebten Zone der Abschnitte 4~5 macht 8,0~11,5 % des Gesamtwasservolumens aus, und ein Wasservolumen in inneren und äußeren Bögen einer achten Zone der Richtabschnitte 6, Abschnitt 7 und Abschnitt 8 macht 8,0~11,5 % des Gesamtwasservolumens aus, und ein verbleibendes Wasservolumen wird dem horizontalen Abschnitt zugewiesen.

## Revendications

1. Procédé de production d'ébauches de coulée continue microalliées au V-N exemptes de fissures de surface, **caractérisé en ce que** les ébauches de coulée continue sont produites à partir d'un acier microallié au V-N constitué des composants chimiques suivants en pourcentage en masse : C : 0,09~0,13 %, Si : 0,1~0,4 %, Mn : 1,0~3,0 %, P : ≤ 0,05 %, S : ≤ 0,05 %, V : 0,1∼0,4 %, N : 0,011~0,2 %, le reste étant du Fe et des éléments d'impuretés inévitables ; le procédé comprenant successivement les processus suivants : élaboration au convertisseur, affinage LF et coulée continue ; dans le processus d'élaboration au convertisseur, une proportion de fonte liquide est contrôlée entre 88,0 % en masse et 91,0 % en masse, un mode de soufflage combiné par le haut et par le bas est utilisé tout au long du processus, et de l'azote gazeux est soufflé en premier puis de l'argon gazeux est soufflé ensuite pendant le processus de soufflage, dans lequel une durée de soufflage d'argon n'est pas inférieure à 3 minutes; un alliage de désoxydation est effectué pendant le processus de coulée dans le processus d'élaboration au convertisseur, tandis qu'une filtration du laitier est également effectuée ; un procédé d'opération spécifique de l'alliage de désoxydation est le suivant : pendant le processus de coulée, une substance contenant du silicium est choisie pour la désoxydation avec une quantité d'addition de 3,5~4,0 kg/tonne d'acier ; et des alliages de silicium-manganèse et de vanadium-azote sont choisis pour l'alliage, dans lequel une quantité d'addition de l'alliage de vanadium-azote est de 1~2 kg/tonne d'acier ; l'affinage LF est effectué après la coulée, et l'affinage est sans dégazage sous vide ; dans le processus d'affinage LF, dans une phase initiale de l'affinage LF, une quantité de soufflage d'argon pour l'agitation par soufflage d'argon est de 400-1000 L/minute, une durée d'agitation par soufflage d'argon est de 3-4 minutes, une substance contenant du silicium doit être utilisée pour la désoxydation, et les composants sont ajustés de manière précise sous la condition d'agitation par soufflage d'argon ; dans le processus d'affinage LF, à la fin de l'affinage LF, une quantité de soufflage d'argon pour l'agitation par soufflage d'argon est de 100-200 L/minute, et une durée d'agitation par soufflage d'argon est ≥ 5 minutes ; une durée totale d'affinage est contrôlée dans les limites de 40~50 minutes, et la teneur en N obtenue est de 100-2000 ppm ; dans le processus de coulée continue, une quantité d'eau spécifique dans le processus de coulée continue est de 0,7~1,25 L/kg ; dans le processus de coulée continue, une coulée protégée est adoptée, l'orifice de coulée est fermé immédiatement lorsque la grande poche de coulée émet une alarme à la fin de la coulée, la réouverture de l'orifice de coulée est strictement interdite après la fermeture de l'orifice de coulée, une poche intermédiaire est recouverte d'un agent de couverture alcalin, et une lingotière utilise un laitier protecteur pour acier à faible teneur en carbone.

2. Procédé de production selon la revendication 1, **caractérisé en ce qu'**une spécification de section transversale des ébauches de coulée continue est de (150-350) mm * (1250-2400) mm.

3. Procédé de production selon la revendication 1 ou 2, **caractérisé en ce que** dans le processus d'élaboration au convertisseur, le processus de soufflage adopte une méthode de soufflage direct jusqu'au bout sans processus de ressoufflage ; de préférence, une teneur en C au point final d'élaboration est contrôlée entre 0,09 - 0,13 % en masse, et une température de coulée est comprise entre 1625 ~ 1645 °C.

4. Procédé de production selon la revendication 1, **caractérisé en ce que** dans le processus de coulée continue, un degré de surchauffe de l'acier fondu est de 10-25 °C ; de préférence, une vitesse de coulée pendant le processus de coulée continue est de 1,0~1,3 m/minute.

5. Procédé de production selon la revendication 1, **caractérisé en ce que** la filtration du laitier est effectuée en utilisant une substance contenant du CaO avec une quantité d'addition de 3,5~4,0 kg/tonne d'acier, et la substance contenant du CaO doit être ajoutée avant que l'acier fondu n'atteigne les 3/4.

6. Procédé de production selon la revendication 1, **caractérisé en ce que** dans le processus de coulée continue, une distribution spécifique du volume d'eau dans le processus de coulée continue est la suivante : un volume d'eau dans les arcs intérieur et extérieur d'un rouleau de pied grand côté de l'ébauche de coulée continue représente 8,0∼10,0 % du volume d'eau total, un volume d'eau dans un rouleau de pied petit côté représente 3,4~4,5 % du volume d'eau total, un volume d'eau dans les arcs intérieur et extérieur d'une deuxième zone de la section de cintrage vertical représente 11,0~15,9 % du volume d'eau total, un volume d'eau dans les arcs intérieur et extérieur d'une troisième zone représente 13,0~15,9 % du volume d'eau total, un volume d'eau dans les arcs intérieur et extérieur d'une quatrième zone représente 12,0~13,0 % du volume d'eau total, un volume d'eau dans les arcs intérieur et extérieur d'une cinquième zone de la section d'arc 1 représente 8,5~9,5 % du volume d'eau total, un volume d'eau dans les arcs intérieur et extérieur d'une couardise zone correspondant aux sections d'arc 2 et 3 représente 12,0~14,0 % du volume d'eau total, un volume d'eau dans les arcs intérieur et extérieur d'une septième zone des sections 4~5 représente 8,0~11,5 % du volume d'eau total, et un volume d'eau dans les arcs intérieur et extérieur d'une huitième zone des sections de redressage 6, section 7 et section 8 représente 8,0~11,5 % du volume d'eau total, tandis que le volume d'eau restant est alloué à la section horizontale.
